

D. E. Hayward,

Shoe Upner,

No 40,409.

Patented Oct. 27, 1863.

Fig. 2.



Fig. 1.



Witnesses:

Sam. Cooper  
John Schenck

Inventor:

D. E. Hayward

# UNITED STATES PATENT OFFICE.

DANIEL E. HAYWARD, OF MELROSE, MASSACHUSETTS.

## IMPROVED HEEL STIFFENER OR COUNTER FOR BOOTS AND SHOES.

Specification forming part of Letters Patent No. 40,409, dated October 27, 1863.

*To all whom it may concern:*

Be it known that I, DANIEL EDWIN HAYWARD, of Melrose, in the county of Middlesex and State of Massachusetts, have invented an Improved Heel Stiffener or Counter for Boots and Shoes, of which the following is a full, clear, and exact description, reference being had to the accompanying drawings, making part of this specification, in which—

Figure 1 is a view of my improved heel-stiffener; Fig. 2, a view of the piece of sheet rubber of which it is made.

Heel stiffeners or counters have heretofore been made of leather; but this material is costly and the labor required to cut them out and skive them is considerable. The chief objection, however, to which they are liable arises from the time and labor required to apply them to the boot. After being cut out and skived they are temporarily secured to the last and lining and then bent round and crimped over upon the insole and secured there. This must be done while the stiffener is wet and pliable. The leather stiffener is also liable to the objection that it will lose its resiliency if bent out of shape when wet and will not return to its original form, and thus the boot wears over to one side.

The cheaper substitutes for leather which have been employed for stiffeners—such as pasteboard and factitious leather—are valueless.

I am also aware that heel-stiffeners have been made of sheet-rubber, which has been cut, folded, crimped, and cemented over the shoe while in course of construction. This is expensive, and I lay no claim to any such stiffeners.

In the manufacture of my improved stiffener I employ any suitable compound of india-rubber, which, when vulcanized, will have the required stiffness combined with the necessary resiliency. This compound, after being ground upon the ordinary heated rolls, is spread in a sheet of from one-eighth to one-tenth inch in thickness upon cotton or other cloth, the thickness of the sheet and of the cloth varying with the size of the required

stiffener. Pieces, Fig. 2, are then cut from the sheet of cloth and rubber, of the required size, which are placed in a mold and vulcanized, the cloth being thrown upon the inside of the stiffener and the mold being of a form that shall give it the required shape, Fig. 1, the part *f*, which goes beneath the heel, being of the exact form ultimately required, so that when applied to the boot or shoe it is simply necessary to put it in place, no wetting, crimping, bending, or temporary nailing being required. When the upper leather and sole are applied, the stitches, nails, or pegs that hold them together also pass through the part *f* of the stiffener in the ordinary manner. This stiffener also is permanently resilient, even when wet, and does not lose its form or shape, however long or severe the wear to which it is exposed.

This stiffener may be placed outside the leather, if preferred.

The proportions which I prefer for the compound to be employed in the manufacture of my improved counters are as follows: eight pounds crude rubber, two pounds litharge, one pound white lead, one pound lamp-black, four pounds calcined plaster, and six ounces flowers of sulphur. This compound, after being thoroughly ground upon the ordinary heated rolls and placed in the molds, is vulcanized by exposure, for ten hours or thereabout, to a temperature of 275° Fahrenheit. I do not, however, wish to confine myself to any particular compound or to any particular length of time or degree of heat for vulcanizing the same.

What I claim as my invention, and desire to secure by Letters Patent as a new article of manufacture, is—

A heel stiffener or counter, of india-rubber and its compounds, which is shaped and vulcanized in the mold in which it is formed and made, and operating as set forth, for the purpose described.

D. E. HAYWARD.

Witnesses:

SAM. COOPER,  
P. E. TESCHEMACHER.